

# United States Patent [19]

Yasumori et al.

[11] 3,898,672

[45] Aug. 5, 1975

[54] ELECTROSENSITIVE RECORDING

MEMBER

- [75] Inventors: Akiyoshi Yasumori; Katsuichi Ohta, both of Yokohama; Makoto Kunikane, Tokyo; Michiharu Abe, Kawasaki; Shuichi Karasawa, Kokubunji, all of Japan
- [73] Assignee: Ricoh Co., Ltd., Tokyo, Japan
- [22] Filed: June 10, 1974
- [21] Appl. No.: 478,003

Related U.S. Application Data

- [63] Continuation of Ser. No. 324,829, Jan. 18, 1973, abandoned.

[30] Foreign Application Priority Data

Jan. 28, 1972 Japan 47-10897

- [52] U.S. Cl. 346/135; 117/201; 204/2; 252/520
- [51] Int. Cl. G01d 15/34
- [58] Field of Search 346/135, 74 S, 74 SB, 74 SC; 117/201, 221; 204/2; 252/507, 518, 520

[56]

References Cited

UNITED STATES PATENTS

|           |        |                   |           |
|-----------|--------|-------------------|-----------|
| 2,294,149 | 8/1942 | Kline et al. .... | 346/135   |
| 2,940,941 | 6/1960 | Dalton .....      | 252/520 X |
| 3,138,547 | 6/1964 | Clark .....       | 204/2     |
| 3,245,833 | 4/1966 | Trevoy .....      | 117/201   |
| 3,263,604 | 8/1966 | Dalton .....      | 346/135 X |
| 3,516,911 | 6/1970 | Hopps .....       | 204/2     |
| 3,684,746 | 8/1972 | Juna et al. ....  | 252/507   |

Primary Examiner—Joseph W. Hartary

Attorney, Agent, or Firm—Cooper, Dunham, Clark, Griffin & Moran

[57]

ABSTRACT

Electrosensitive recording member in which blackish pattern is electrically formed on a recording layer by sparking between a needle-like electrode (stylus) and the recording layer comprising a binder and an electrically reducible metal compound. Copper iodide (CuI) is specifically included in the recording layer to increase its electroconductivity.

6 Claims, 3 Drawing Figures



PATENTED AUG 5 1975

3,898,672

FIG. 1



FIG. 2



FIG. 3



## ELECTROSENSITIVE RECORDING MEMBER

This is a continuation of application Ser. No. 324,829 filed Jan. 18, 1973, now abandoned.

## BACKGROUND OF THE INVENTION

Dry recording members are well known. They are prepared by applying an electrically destructive substance on an electroconductive support having an electroconductive layer such as carbon. The electrically destructive substance is, for example, a synthetic resin. In the dry recording members the electroconductive layer functions as one electrode, and the other electrode is a metallic needle-like electrode (stylus) which contacts the layer of electrically destructive substance. By applying a D.C. or A.C. voltage, for example 100-150V, between the two electrodes separated by the destructive substance layer, an electric current (10-20mA) flows and consequently the destructive layer is broken down and the carbon black layer appears. The needle-like electrode (stylus) is moved while contacting the electrically destructive layer. The pattern of the carbon black is formed on the support by controlled tracing of the stylus. The dry recording member is used in the field of a facsimile recording. However, dry recording members have several shortcomings. For example, (1) they may not be sufficiently sensitive; (2) when the voltage is applied, an offensive odor is emitted as a result of the combustion of the electrically destructive substance; (3) they may be undesirable sparking and breakdown of the recording member caused by increasing the voltage in order to speed up the recording.

Substitutes for the above described dry recording members have been proposed and disclosed, for example, in U.S. Pat. Nos. 3,138,547 and No. 3,516,911. In the proposed substitutes, the electroinsensitive recording members consist essentially of a recording layer formed on an electroconductive support. The recording layer comprises a mixture of powder of an electrically reducible metal compound such as ZnO, SnO<sub>2</sub>, TiO<sub>2</sub>, Bi<sub>2</sub>O<sub>3</sub>, V<sub>2</sub>O<sub>5</sub>, Sb<sub>2</sub>S<sub>3</sub>, or H<sub>2</sub>MoO<sub>4</sub>, and a synthetic resin binder such as synthetic rubber or ethyl cellulose. The electroconductive support is, for example, a metallic foil or an electroconductive plastic film. These electroinsensitive recording members may be used in the same manner as the described dry recording members. A blackish pattern is formed on the recording layer by tracing of the stylus.

An object of the present invention is to provide improved electroinsensitive recording members. The recording members of the present invention are characterized by the low resistance of the recording layer. Therefore, a nonconductive support may be utilized and consequently, the recording member can be provided inexpensively. Further, vivid black patterns of high density can be formed on the recording layer.

## SUMMARY OF THE INVENTION

The electroinsensitive recording members of this invention are made up of a support and an electroinsensitive recording layer formed on a surface of the support. The electroinsensitive recording layer is a thin layer comprising an organic binder, an electrically reducible metal compound and copper iodide (CuI). CuI is an electroconductivity-increasing substance. The metal compound and CuI are uniformly dispersed in the binder. As a result, the electroinsensitive recording mem-

bers of the invention all have an electroinsensitive recording layer with a high electroconductivity. Accordingly, the electroinsensitive recording members of this invention are characterized in that: (1) a nonconductive support may be utilized (the use of an electroconductive support is not necessarily required), and (2) a vivid pattern of high density can be formed on the electroinsensitive recording layer at high recording speed by applying a relatively low voltage. A nonconductive support such as paper or plastic film is inexpensive in comparison with an electroconductive support such as aluminum foil or aluminum-coated paper. This is a feature of the present invention. However, an electroinsensitive recording layer containing CuI in accordance with this invention may be formed on the electroconductive support.

The electrically reducible metal compounds which may be used in forming an electroinsensitive recording layer of the invention are as follows: zinc oxide (ZnO), 20 cadmium oxide (CdO), barium oxide (BaO), tin oxide (SnO<sub>2</sub>), lead oxide (PbO, Pb<sub>2</sub>O<sub>3</sub>, PbO<sub>2</sub>), titanium oxide (TiO<sub>2</sub>), zirconium oxide (ZrO<sub>2</sub>), antimony oxide (Sb<sub>2</sub>O<sub>3</sub>, Sb<sub>2</sub>O<sub>5</sub>, Pb<sub>2</sub>O<sub>5</sub>), bismuth oxide (Bi<sub>2</sub>O<sub>3</sub>, Bi<sub>2</sub>O<sub>4</sub>, Bi<sub>2</sub>O<sub>5</sub>), vanadium oxide (V<sub>2</sub>O<sub>5</sub>), molybdenum oxide (MoO<sub>3</sub>), tungsten oxide (WO<sub>3</sub>), cerium oxide (CeO<sub>2</sub>), 25 molybdcic acid (H<sub>2</sub>MoO<sub>4</sub>), tungstic acid (H<sub>2</sub>WO<sub>4</sub>), molybdates (Na<sub>2</sub>MoO<sub>4</sub>, K<sub>2</sub>MoO<sub>4</sub>, CaMoO<sub>4</sub>, PbMoO<sub>4</sub>, (NH<sub>4</sub>)<sub>2</sub>MoO<sub>4</sub>, (NH<sub>4</sub>)<sub>6</sub>Mo<sub>7</sub>O<sub>24</sub>.4H<sub>2</sub>O, Na<sub>2</sub>Mo<sub>8</sub>O<sub>25</sub>.17H<sub>2</sub>O, (NH<sub>4</sub>)<sub>6</sub>[CrMo<sub>12</sub>O<sub>42</sub>].2H<sub>2</sub>O), molybdsilicic acid 30 (H<sub>4</sub>[SiO<sub>4</sub>Mo<sub>12</sub>O<sub>36</sub>]), molybdophosphoric acid (H<sub>3</sub>[PO<sub>4</sub>Mo<sub>12</sub>O<sub>36</sub>]), tungstophosphoric acid (H<sub>3</sub>[PO<sub>4</sub>W<sub>12</sub>O<sub>36</sub>]), cobalt oxides Co<sub>2</sub>O<sub>3</sub>, Co<sub>3</sub>O<sub>4</sub>), mercury oxide (HgO), chromium oxide (Cr<sub>2</sub>O<sub>3</sub>), niobium oxide (Nb<sub>2</sub>O<sub>5</sub>), tantalum oxide (Ta<sub>2</sub>O<sub>5</sub>), manganese oxide 35 (MnO<sub>2</sub>), antimonic acid (HSbO<sub>3</sub>, H<sub>3</sub>SbO<sub>4</sub>), stannic acid (SnO<sub>2</sub>.xH<sub>2</sub>O), titanic acid (H<sub>4</sub>TiO<sub>4</sub>, H<sub>2</sub>TiO<sub>3</sub>) vanadic acid (HVO<sub>3</sub>), selenic acid (H<sub>2</sub>SeO<sub>4</sub>), bismuthate (NaBiO<sub>3</sub>), zinc sulfide (ZnS) and antimony sulfide (Sb<sub>2</sub>S<sub>5</sub>).

40 Among the above-cited metal compounds, ZnO, TiO<sub>2</sub>, V<sub>2</sub>O<sub>5</sub>, H<sub>2</sub>MoO<sub>4</sub>, H<sub>2</sub>WO<sub>4</sub> and (NH<sub>4</sub>)<sub>6</sub>Mo<sub>7</sub>O<sub>24</sub>.4H<sub>2</sub>O are preferred.

The following organic compounds may preferably be 45 used as a nonconductive binder: polyvinyl alcohol, polyvinyl acetate, polyvinyl chloride, ethyl cellulose, gelatin, butadiene-styrene copolymers, vinyl acetate-crotonic acid copolymers, polymethylmethacrylate, polyethylmethacrylate and the like.

Preferred solvents for use in dissolving the binder are 50 as follows: water, ammonia water, toluene, xylene, methyl ethyl ketone, methyl isobutyl ketone, cyclohexane, alcohols such as methyl alcohol and ethyl alcohol, aliphatic hydrocarbon such as petroleum solvents and isoparaffinic solvents.

55 Paper or plastic films are the preferred nonconductive supports. However, electroconductive supports, for example, metal-coated sheets such as aluminum-coated paper or film and metal foils such as aluminum foil may be used.

The electroinsensitive recording layers of the present invention contain one part by weight of binder with 60 from 5 to 10 parts by weight of a mixture of CuI and at least one of the above-cited electrically reducible metal compounds dispersed therin.

65 The electrically reducible metal compound and CuI are preferably used in the ratio of from 1 to 10 parts by weight of CuI per one part by weight of the electrically

reducible metal compound. However, the amount of CuI used may be up to 30 parts by weight per one part by weight of the metal compound.

Certain embodiments of the invention are illustrated in the accompanying drawings in which:

FIG. 1 is a cross section of one form of the invention using a paper as a nonconductive support.

FIG. 2 is a cross section of a modification of the invention using a metal-coated paper as an electroconductive support.

FIG. 3 shows the method of recording on an electro-sensitive recording layer prepared in accordance with the invention.

The FIGURES show the thickness of the paper and the coating layer thereon enlarged as compared with their actual thickness, for the sake of clarity of illustration.

A binder selected from amongst the above-cited organic binders is dissolved in a solvent and to this solution is added at least one of the electrically reducible metal compounds and CuI in the above-mentioned ratio. The resulting mixture is dispersed or suspended by ball milling to produce a homogeneous dispersion of the metal compound and CuI in a solution of the binder. The resulting dispersion is applied onto a surface of paper 1 by means of e.g. a wire-bar and then dried at a temperature of about 100°C to form an electro-sensitive recording layer 2 on the surface of the paper 1. The preferred thickness of the recording layer is from about 5 to about 100 $\mu$ . Alternatively, as shown FIG. 2, an electro-sensitive recording layer 2 may be formed on a metal-coating 3 of a metal-coated paper 1.

Referring to FIG. 3, the electro-sensitive recording member thus obtained is placed on a flat plate 4 and a D.C. or an A.C. voltage of from 50 to 200V is applied to a stylus 5 and a lead wire 6 and the stylus is traced at a speed of from 25 – 400 m/min. in light contact with the recording layer 2. A current of from 5 to 200 mAmp. flows between the stylus 5 and the recording layer 2 and the passage of the current causes the metal compound to become reduced to a dark compound in color contrast with the surrounding unreduced portions of the electro-sensitive recording layer. A vivid blackish pattern is formed according to the tracings of the stylus.

#### DESCRIPTION OF THE PREFERRED EMBODIMENTS

The following nonlimiting examples are given by way of illustration only.

#### EXAMPLE 1

A dispersion for use in forming an electro-sensitive recording layer was prepared from the following ingredients:

|                   |       |
|-------------------|-------|
| $H_2MoO_4$        | 20g   |
| CuI               | 100g  |
| Butadiene-styrene | 15g   |
| copolymer         |       |
| Toluene           | 100ml |

Butadiene-styrene copolymer was dissolved in toluene, and to this solution was added  $H_2MoO_4$  and CuI. This mixture was dispersed by ball milling for about 24 hours. The homogeneous dispersion thus produced was applied onto a surface of paper by means of a wire-bar and then dried at a temperature of about 100°C to obtain an electro-sensitive recording member with a light yellowish recording layer 10  $\mu$  thick. The sheet resistance of this recording layer was  $10^3 \Omega/\text{square}$ . Utilizing the electro-sensitive recording member thus prepared, a pattern was produced, in the manner as shown in FIG. 3, under the following conditions:

|                        |                                                                              |
|------------------------|------------------------------------------------------------------------------|
| Recording device used  | "Toshafax" (trade name of a recording device; sold by Tokyo Kooku Keiki Co.) |
| Applied voltage        | D.C. 100V<br>(Stylus in positive electrode)                                  |
| Moving speed of stylus | 100 m/min.                                                                   |

25 A vivid greenish black pattern having a density of 1.3 was produced on the recording layer. The density was measured by means of "Macbeth Densitometer RD-400" sold by Macbeth Institute.

30 For comparison, a control electro-sensitive recording member was prepared by the same procedure except that 120g of  $H_2MoO_4$  was used in place of 20g of  $H_2MoO_4$  and 100g of CuI. The sheet resistance of the recording layer thus produced was about  $10^8 \Omega/\text{square}$ . The same procedure mentioned above was repeated to form a pattern except that a D.C. voltage of 200V was applied instead of 100V. However, no pattern could be produced.

35 Another control electro-sensitive recording member containing CuI was prepared by the above procedure except that aluminum-coated paper was utilized as a support in place of paper. The recording member thus prepared gave a blackish pattern having a density of 1.0 at a D.C. voltage of 80V and stylus speed of 160 m/min. It is apparent from this example that the products of 40 this invention can give a vivid pattern even when the stylus is moved at a relatively high moving speed.

#### EXAMPLE 2 – EXAMPLE 10

45 Electro-sensitive recording members No. 2 – No. 10 were prepared by repeating the procedure of Example 1 except that metal compounds, binders and solvents shown in the table below were used. In these Examples, paper was used as a support.

A pattern was produced on each of the recording members No. 2 – No. 10 in the same manner as Example 1, and the pattern thus obtained was evaluated. The data and the results are shown in the table below:

| Example No | Metal Compound (g) | CuI (g) | Binder (g)                            | Solvent (ml)         | Applied voltage (V) | Pattern Color  | Pattern Density |
|------------|--------------------|---------|---------------------------------------|----------------------|---------------------|----------------|-----------------|
| 2          | $H_2MoO_4$<br>20   | 60      | Ethyl cellulose<br>10                 | Ethyl alcohol<br>70  | D.C.<br>100         | Greenish black | 1.2             |
| 3          | $H_2MoO_4$<br>20   | 20      | Vinyl acetate-crotonic acid copolymer | Methyl alcohol<br>50 | D.C.<br>100         | Black          | 1.0             |

Table - Continued

| Example No | Metal Compound (g)                                                                                        | CuI (g) | Binder (g)                               | Solvent (ml)      | Applied voltage (V) | Pattern        | Color | Density |
|------------|-----------------------------------------------------------------------------------------------------------|---------|------------------------------------------|-------------------|---------------------|----------------|-------|---------|
| 4          | K <sub>2</sub> MoO <sub>4</sub>                                                                           |         | Butadiene-Styrene copolymer 15           | Toluene 100       | D.C. 200            | Greenish Brown | 0.8   |         |
|            |                                                                                                           | 20      | 100                                      |                   |                     |                |       |         |
| 5          | H <sub>2</sub> WO <sub>4</sub>                                                                            |         | Vinyl acetate-crotonic acid copolymer 5  | Methyl alcohol 50 | D.C. 100            | Black          | 1.0   |         |
|            |                                                                                                           | 20      | 20                                       |                   |                     |                |       |         |
| 6          | (NH <sub>4</sub> ) <sub>6</sub> Mo <sub>7</sub> O <sub>24</sub> ·4H <sub>2</sub> O                        |         | Vinyl acetate-crotonic acid copolymer 5  | Methyl alcohol 50 | D.C. 100            | Black          | 1.0   |         |
|            |                                                                                                           | 20      | 20                                       |                   |                     |                |       |         |
| 7          | V <sub>2</sub> O <sub>5</sub>                                                                             |         | Polyvinyl alcohol 5                      | Water 50          | D.C. 100            | Black          | 1.3   |         |
|            |                                                                                                           | 20      | 30                                       |                   |                     |                |       |         |
| 8          | ZnO                                                                                                       |         | Vinyl acetate-crotonic acid copolymer 10 | Methyl alcohol 70 | D.C. 100            | Brownish black | 0.8   |         |
|            |                                                                                                           | 20      | 40                                       |                   |                     |                |       |         |
| 9          | ZnO 10 H <sub>2</sub> MoO <sub>4</sub> 10                                                                 | 40      | Butadiene-styrene copolymer 10           | Toluene 70        | D.C. 100            | Black          | 1.0   |         |
|            |                                                                                                           | 10      |                                          |                   |                     |                |       |         |
| 10         | TiO <sub>2</sub> 10 (NH <sub>4</sub> ) <sub>6</sub> Mo <sub>7</sub> O <sub>24</sub> ·4H <sub>2</sub> O 10 | 40      | Butadiene-styrene copolymer 10           | Toluene 70        | D.C. 100            | Bluish black   | 0.7   |         |
|            |                                                                                                           | 10      |                                          |                   |                     |                |       |         |

As is seen from the above-mentioned data, preferred electroinsensitive recording members can be obtained by forming an electroinsensitive recording layer containing CuI in an amount of from 1 to 10 parts by weight of CuI per one part by weight of an electrically reducible metal compound on a nonconductive support. When said electroinsensitive recording layer containing CuI is formed on an electroconductive support such as aluminum foil or aluminum-coated paper, a good pattern of high density can be produced at relatively low voltage even when the stylus is moved.

We claim:

1. An electroinsensitive recording member comprising a nonconductive support and an electroinsensitive recording layer formed on the support, said electroinsensitive recording layer containing a binder having a mixture of an electrically reducible metal compound and copper iodide (CuI) dispersed therein; the weight ratio of mixture to binder being from 5:1 to 10:1.

2. An electroinsensitive recording member of claim 1 in which said mixture of an electrically reducible metal compound and copper iodide is a mixture of one part by weight of the electrically reducible metal compound and from 1 to 10 parts by weight of copper iodide.

3. An electroinsensitive recording member of claim 1 in which said electrically reducible metal compound is one selected from the group consisting of ZnO, TiO<sub>2</sub>, V<sub>2</sub>O<sub>5</sub>, H<sub>2</sub>MoO<sub>4</sub>, H<sub>2</sub>WO<sub>4</sub> and (NH<sub>4</sub>)<sub>6</sub>Mo<sub>7</sub>O<sub>24</sub>·4H<sub>2</sub>O.

4. An electroinsensitive recording member of claim 1 wherein the nonconductive support is paper.

5. An electroinsensitive recording member of claim 1 wherein the nonconductive support is a plastic.

6. An electroinsensitive recording member of claim 1 in which said mixture of an electrically reducible metal compound in copper iodide is a mixture of 1 part by weight of the electrically reducible metal compound and from 1 to 10 parts by weight of copper iodide.

50 \* \* \* \* \*